

1

3,337,377

**PROCESS FOR THE TREATMENT OF MAGNESIUM-SILICON ALUMINUM ALLOYS**

Jacques Bonnarin, La Motte-Servolex, France, assignor to Pechiney, Compagnie de Produits Chimiques et Electrometallurgiques, Paris, France  
No Drawing. Filed Dec. 18, 1963, Ser. No. 331,381  
Claims priority, application France, Dec. 20, 1962,  
919,280

4 Claims. (Cl. 148—159)

The present invention has for its object a process which makes it possible to improve the characteristics of aluminum alloys containing magnesium and silicon. The invention also relates to the alloys obtained by carrying this process into effect.

It is well known that the aluminum alloys which contain magnesium and silicon are capable of being given improved mechanical properties by quenching from a temperature at which the metal is entirely or almost entirely in the state of solid solution. This rapid cooling is then followed by a natural or artificial aging. Such alloys are employed either in the cast state or in the transformed state obtained by operations resulting from hot working or cold working, such as forging, forming, rolling, extruding, drawing and wire-drawing.

The mechanical characteristics obtained after quenching and artificial aging, or tempering, are proportionally higher for a quenching of given intensity when the time elapsed between these two operations is shorter. It is only in the case where a cold-hardening operation is immediately followed by an air quenching that this disadvantage is no longer observed, but then only reduced mechanical characteristics are obtained.

These facts constitute serious disadvantages for industrial production because it is frequently difficult to organize the production operations in such a way that the annealing immediately follows the quenching. It is even desirable in certain cases to take advantage of the plasticity imparted to the alloy by the quenching in order to shape it before causing it to be hardened by the annealing. In the second case, the necessity of quenching in air immediately after the cold-hardening operation is more readily accepted, but the reduction of the mechanical characteristics still represents a serious disadvantage.

In order to overcome these disadvantages, special and frequently troublesome thermal treatments have been proposed. One of these consists in modifying the annealing conditions, but it necessitates special installations, while another consists in causing billets to be subjected to a previous homogenization treatment at a temperature in the region of 600° C. before any deformation.

The present invention has for its object a process for

2

improving aluminum alloys containing magnesium and silicon, which makes it possible to reduce to a considerable extent the effect of the waiting between the quenching and annealing operations. In the case of an air quenching 5 immediately following a cold-working operation, the instant invention has the effect of avoiding any reduction in the mechanical properties without it being necessary either to modify the thermal treatment or to provide a previous homogenization treatment.

Another object of the invention is the provision of an alloy obtained by using the above process.

These and other objects of this invention will appear hereinafter and it will be understood that the specific embodiments hereinafter set forth are provided solely for purposes of illustration and not by way of limitation.

In the process according to the invention, a quantity of tin between 0.001 and 0.1 percent and preferably between 0.005 and 0.1 percent is added to the aluminum alloy containing magnesium and silicon. Typical alloys according to the invention have the following compositions:

magnesium—0.2 to 2%.  
silicon—0.2 to 5%.

tin—0.001 to 0.1%.

25 impurities—iron up to 0.5%, others up to 0.2% each, with the total being less than 1%.

aluminum—balance.

Preferred alloys which are modified in accordance with the instant invention have the following compositions:

30 magnesium—0.4 to 1.0%.

silicon—0.4 to 1.8%.

tin—0.005 to 0.1%.

35 impurities—iron up to 0.5%, others up to 0.2% each with the total being less than 1%.

aluminum—balance.

The alloys referred to in the following examples were characterized by compositions falling within the above ranges.

40 In order to be able best to understand the subject of the invention, there is considered the case of an alloy which has undergone an extruding operation. An aluminum alloy containing magnesium and silicon, extruded and quenched in air on leaving the press, is not sensitive to the waiting time between the quenching and the annealing. On the contrary, if it has not been subjected to previous homogenization, it only has mediocre characteristics.

45 An addition of tin then has the effect of increasing the mechanical characteristics thereof and makes it possible to obtain, without previous homogenization, characteristics which are at least equal to those which are provided by the alloys homogenized before extrusion.

TABLE NO. 1  
NONHOMOGENIZED BILLETS

| Aging                        | Alloy A |      |    | Alloy A+0.01% Sn |      |    |
|------------------------------|---------|------|----|------------------|------|----|
|                              | E       | R    | A  | E                | R    | A  |
| After aging for 15 days      | 6.3     | 10.7 | 15 | 8.3              | 13.9 | 15 |
| Tempering—8 hrs. at 175° C.: |         |      |    |                  |      |    |
| 1 day after quenching        | 15      | 18   | 11 | 18.6             | 21.7 | 19 |
| 1 month after quenching      | 13.9    | 17.8 | 14 | 18.8             | 24.8 | 14 |

HOMOGENIZED BILLETS

|                              |      |      |    |      |      |    |
|------------------------------|------|------|----|------|------|----|
| After aging for 15 days      | 7.7  | 12.5 | 13 | 8.7  | 15.2 | 19 |
| Tempering—8 hrs. at 175° C.: |      |      |    |      |      |    |
| 1 day after quenching        | 21.6 | 24.2 | 13 | 20.8 | 24.3 | 12 |
| 1 month after quenching      | 21.8 | 24.8 | 14 | 21.1 | 25.2 | 16 |

E—The elastic limit in kg./mm.<sup>2</sup> (0.2 percent offset).

R—Ultimate strength in kg./mm.<sup>2</sup>

A—Percent elongation at rupture.

It is shown from this table that:

(a) The alloy is insensitive to the waiting time between quenching and the annealing;

(b) The addition of a quantity of tin as small as 0.01% causes a considerable improvement in the mechanical characteristics of the non-homogenized alloy.

An alloy of the type referred to, when extruded and quenched in water or oil just after leaving the press is very sensitive to the waiting time between the quenching and the annealing. The addition of tin overcomes this disadvantage.

As a particular example, tin is added in amounts of 0.01 percent and 0.1 percent to an alloy, the composition of which is as follows:

|           | percent |
|-----------|---------|
| Magnesium | 0.81    |
| Silicon   | 0.60    |
| Iron      | 0.34    |

The alloy to which no tin is added and the two alloys containing the addition are cast into billets, then extruded under the same conditions without previous homogenization of the billets. The bars which are obtained are heated for two hours to 560° C., and then quenched in water. They are then subjected to an annealing operation which lasts 10 hours at a temperature of 175° C. The annealing is conducted either immediately after the quenching or after an increasingly long period of time.

The results of the traction test are given by Table No. 2 in which the notations are those which have been set out in respect of Table No. 1.

TABLE NO. 2

| Time*        | Alloy B |      |    | Alloy B+0.01%Sn |      |    | Alloy B+0.1% Sn |      |    |
|--------------|---------|------|----|-----------------|------|----|-----------------|------|----|
|              | E       | R    | A  | E               | R    | A  | E               | R    | A  |
| 0.....       | 28.3    | 31.6 | 11 | 31              | 33.8 | 10 | 29.9            | 33.2 | 7  |
| 4 hrs.....   | 25.3    | 29.2 | 12 | 31              | 33.8 | 10 | 30.9            | 33.9 | 5  |
| 4 days.....  | 22.7    | 27.5 | 14 | 27.1            | 32.1 | 11 | 28              | 31.6 | 11 |
| 15 days..... | 22.5    | 28   | 13 | 27.3            | 32.6 | 11 | 26.6            | 31   | 10 |

It is shown from this table that:

(a) For the alloy B without additive, the mechanical characteristics are greatly reduced when the waiting time between the quenching and the annealing is increased. The effect is very marked, even for short waiting times, of the order of a few hours.

(b) The addition of the optimum amounts of tin specified to the alloys in question provides highly significant improvements even where the waiting time between quenching and annealing is of the order of 15 days. These improvements are most apparent when considering the mechanical properties set forth in the above table.

The tin can be introduced into the alloys by means of direct additions, through the use of master alloys or by means of compounds which will decompose to the extent that the tin will be free for its intended function.

The additions specified in accordance with this invention are suitable for use in combination with a wide variety of aluminum-magnesium-silicon alloys. The fol-

lowing comprises a list of additional elements which may be included in such alloys and which will not affect the improvements provided by the tin additions:

|             | Percent by weight, up to |
|-------------|--------------------------|
| 5 Manganese | 6                        |
| Chromium    | 6                        |
| Titanium    | 1                        |
| Zirconium   | 1                        |
| Vanadium    | 1                        |
| 10 Boron    | 0.1                      |

It will also be understood that other additions can be tolerated in alloys of the type described. Thus, alloying elements which are employed in conventional practice for modifying transformation temperatures or for otherwise affecting the mechanical properties of the alloys can be utilized. It will be apparent, however, that such additions are contemplated only where they do not interfere with the function of the tin additions described herein.

20 It will be understood that various changes and modifications can be made in the processes and alloys described which provide the characteristics of this invention without departing from the spirit thereof particularly as defined in the following claims.

25 What is claimed is:

1. In a process for the treatment of aluminum base alloys including the steps of subjecting the alloys to a solution heat treatment, and thereafter aging the alloys, said alloys consisting essentially of from 0.2 to 2.0 percent by weight magnesium and from 0.2 to 5.0 percent by weight silicon, and the balance aluminum, said alloys being subject to losses in mechanical properties due to delays between said solution heat treatment and aging, the improvement in combination therewith including tin 35 in said alloys in an amount between 0.001 and 0.1 percent by weight.

2. A process in accordance with claim 1 wherein magnesium is present in said alloys in amounts between 0.4 and 1.0 percent by weight, silicon is present in said alloys in amounts between 0.4 and 0.8 percent by weight, and iron is present in said alloys in amounts up to 0.5 percent by weight.

3. A process in accordance with claim 1 wherein said alloys contain up to 6 percent by weight manganese, up to 6 percent by weight chromium, up to 1 percent by weight titanium, up to 1 percent by weight zirconium, up to 1 percent by weight vanadium and up to 0.1 percent by weight boron.

4. A process in accordance with claim 1 wherein said tin is included in an amount between 0.005 and 0.1 percent by weight.

#### References Cited

#### UNITED STATES PATENTS

55 2,076,587 4/1937 Kempf et al. ----- 75—147  
2,081,951 6/1937 Paine et al. ----- 75—147

DAVID L. RECK, Primary Examiner.

60 HYLAND BIZOT, Examiner.

R. O. DEAN, Assistant Examiner.